

July 17, 1934.

A. L. BOEGEHOOLD ET AL

1,967,077

PROCESS OF CARBURIZING BRAKE DRUMS

Filed July 13, 1932



Inventors  
Alfred L. Boegehold  
Clarence J. Bobin &  
Clarence F. Smart.

By Blackworn, Spencer & Fluit  
Attorneys

## UNITED STATES PATENT OFFICE

1,967,077

## PROCESS OF CARBURIZING BRAKE DRUMS

Alfred L. Boegehold, Birmingham, Clarence J. Tobin, Detroit, and Clarence F. Smart, Pontiac, Mich., assignors to General Motors Research Corporation, Detroit, Mich., a corporation of Delaware

Application July 13, 1932, Serial No. 622,266

5 Claims. (Cl. 29—152.2)

This invention relates to brake drums, particularly to such drums as are used on motor vehicles.

An object of the invention is to produce a non-scoring drum, one having a high degree of concentricity, and to make such a drum by a simple and inexpensive process.

Another object is to perform upon a drum cold formed from low carbon steel such operations as to avoid the necessity for subsequent machining to obtain concentricity and to provide for non-scoring characteristics.

Other objects and advantages will be understood from the following description.

15 Fig. 1 of the accompanying drawing shows in transverse section a drum after the first forming step of the operation.

Fig. 2 illustrates in vertical section a container having drums about to be carburized.

20 Fig. 3 shows in transverse section a drum after being carburized.

Fig. 4 illustrates in vertical section the final sizing step.

Fig. 5 illustrates in vertical section a portion 25 of the finished drum.

Fig. 6 is a perspective of a drum disclosing a slight modification.

Modern automobiles require brake drums having non-scoring characteristics and having a 30 high degree of concentricity since they are subjected to severe braking pressure.

The process of making drums from low carbon steel by cold forming is well known. Such drums become highly strained in the forming process.

35 Unless this strained condition is relieved by annealing it prevents the attainment of the required high degree of concentricity of the braking surface without resort to a machining operation. Even when the braking surface of such 40 a drum is made concentric by machining, it has a tendency to go out of round in service due to residual strains.

If the cold formed drum is annealed to remove the strains set up during the forming process and thereafter restruck in a die, the drum can be sized to a greater degree of concentricity.

45 Such cold formed steel drums are, however, not sufficiently resistant to scoring to meet the severe braking conditions in modern automobiles. 50 Therefore, it is desirable to raise the carbon content of the braking surface of the drum. This may be done by the known method of heating the drum with solid carbonaceous material or by gas carburizing. If this operation be substituted for the above-mentioned annealing opera-

tion, two results are accomplished. The cold forming strains are removed and the braking surface is transformed into one having high carbon steel. After this dual operation the drum may be sized by striking in a die to secure the 60 required high degree of concentricity so that it is not out of round more than .005" and will remain round in service.

In carrying out the above operation it is found that the initial forming step should bring the 65 drum diameter to .005" less than that of the finished drum. The punch for the final sizing should be of a diameter equal to the desired inside diameter of the finished drum, or .005" 70 larger than the inside diameter of the initially formed drum. This produces a slight stretching of the drum during the final sizing step. The sizing operation should also include the formation of a bead in the back of the drum to remove any distortion in this part of the drum 75 resulting from the second step in the process.

Owing to the elimination of a machining step to produce concentricity, it is possible to reserve for use as a braking surface the outermost layer 80 of the carburized surface which has been found to have preferred frictional and score-resisting characteristics as compared to that layer slightly below the surface. The surface of steel which has been carburized contains a considerably 85 higher concentration of the intensely hard iron carbide than is present at a depth of .010" below the surface.

It has been found that for certain lining materials the drum structure at predetermined 90 depths below the surface may be preferred to the actual surface obtained by carburizing. For such linings it may be desired to machine the drum surface to reach the desired depth. If the drum is not to a high degree concentric, that 95 machining operation will remove more metal in some places than in others with the result that the braking surface lacks uniformity. For this reason the above described forming operation is very much to be desired since at any depth the machining operation will produce a uniform 100 surface.

This novel process, then, is a simple inexpensive way to make a light, non-scoring concentric drum without resort to the use of cast iron; without resort to costly non-scoring alloys; and without resort to the process of adding non-scoring liners to previously formed drums. The new process comprises essentially three steps—(a) forming the drum to a slight under size; (b) a 105 simultaneous carburizing and annealing step; 110

and (c) a final sizing step. Between the second and third steps the drum is preferably cooled slowly rather than quenched. In this way case hardening is prevented.

5 The drawing shows the several steps and the operation. In Fig. 1 is a drum 9 of conventional shape having a flange 11, and preferably formed with a hole 13 in its back wall. This drum has been cold formed from low carbon plain or alloy steel having good cold forming properties. The inner diameter of the drum is very slightly less than that of the finished drum. Several of such drums are then subjected to the second step. To carburize the shoe-engaging surface only of the drum the remaining surface may be protected from the carburizing process. To that end a plate 15 may be placed in the bottom of each drum leaving a space 17 between the plate and the bottom of the drum. Each drum is then filled with carburizing compound 19 and covered with a plate 21. A series of such drums is then assembled on supports 25 within a heat resistant container 23 which is then subjected to heat. The heat converts to a high carbon content the annular surface in contact with the carbonaceous material. The gases may escape to the space beneath the plates 15 and out through the holes 13 and around the outer surface of the drum. As a result of this treatment the annular surface which is to be 30 subject to the frictional contact of the brake shoes is converted to high carbon steel and the rest of the drum retains its low carbon characteristics.

If desired the conversion of the annular braking surface of the drum to high carbon steel may be done by the gas carburizing process. To effect local carburization by this process, the drum after the first forming operation would be copper plated all over and then ground or machined on the 40 braking surface to remove the copper plate. The drum would then be heated in a gaseous carburizing atmosphere which would increase the carbon content of the drum at the braking surface only.

45 The drums are then allowed to cool at a comparatively slow rate which will develop in the high carbon layer a surface composed essentially of lamellar pearlite with or without some free cementite. The heating process simultaneously removes the strained condition produced in the drum during the original forming process. In consequence, the friction surface is non-scoring and the removal of the strains avoids the danger of the drum going out of round in service.

55 For the final sizing step a die 29 is used with a punch 31 to slightly stretch the drum from its under size, as shown by dotted lines, to its final size, as shown by full lines in Fig. 4. Also, the die and punch are shaped to form a bead 33 which is intended to take up the slack or to provide space for the reception of the material caused by the distortion produced in the carburizing step and shown at 27 in Fig. 3.

The configuration of this bead is immaterial. 65 It may be radial, as shown in Fig. 5, or it may be annular, as shown at 35 in Fig. 6.

The brake drum made by the above-described simple process possesses the desired characteristics of hot formed high carbon or special alloy 70 steel drums without the known attendant disadvantages of such drums. Among these disadvantages may be mentioned—

a. The cost of material.

b. The excessive die upkeep cost.  
c. Difficulty of obtaining accurate size.  
d. The necessity for additional cleaning operations.

80 e. Surface decarburization which must be removed by machining to obtain the desired resistance to scoring.

Drums made by the herein described new process possess score-resisting characteristics better than may be obtained in cold formed drums made from steel of intermediate carbon content.

85 Drums made from this new process are relieved from the stresses of the cold forming operations, so that the usual difficulties of obtaining and maintaining a true shape in cold formed drums are minimized.

90 While drums made by this process may be used as they come from the third step of the operations, if it should be necessary to render such drums adaptable to special brake linings, they may obviously be ground or machined or rolled for such purpose.

95 Furthermore, this novel process involves saving of time in manufacture because carburization is effected on a limited surface only, which permits the absence of poor heat-conducting material between the container and the drum enabling the drum to reach the carburizing temperature very quickly.

100 We claim:

105 1. The method of making brake drums which consists in cold forming a drum from sheet metal to a diameter slightly less than that of the finished drum, simultaneously annealing the formed drum and carburizing its friction surface only, and striking the carburized drum in a die to finished dimensions.

110 2. The method of making a brake drum which consists in cold forming a drum of low carbon sheet steel to a diameter slightly less than that of the finished drum, annealing the drum and carburizing its friction surface only, cooling the carburized drum to produce a pearlite surface in the carburized region, and sizing the drum by stretching and shaping it to its desired shape and 115 size.

120 3. The method of making a brake drum which consists in cold forming the drum from sheet material to a size and shape only slightly different from the final shape and size, annealing the drum to remove the strains produced by the forming step and simultaneously carburizing the friction surface only, and thereafter striking the drum in a die to the required final dimensions.

125 4. The process of making carburized brake drums which consists in shaping a blank of sheet material into the form of a drum, forming a hole in the back wall of the drum, covering the back wall with a plate to form a space between the plate and the wall, filling the drum with carbonaceous material, and thereafter heating, whereby the friction surface only is carburized.

130 5. The process of forming brake drums which consists in cold forming the drum from sheet material, annealing the drum and carburizing its 135 shoe-engaging part only, sizing the drum, the sizing step including the forming of a bead in the wall of the drum to take up the distortion produced in the carburizing step.

145

ALFRED L. BOEGEHOOLD.  
CLARENCE J. TOBIN.  
C. F. SMART.